

UNITED STATES PATENT OFFICE

1,923,383

PROCESS OF GRINDING MATERIALS

John H. Lundteigen, Detroit, Mich., assignor to  
The Super Cement Company, a Corporation of  
Michigan

No Drawing. Application January 26, 1929  
Serial No. 335,392

3 Claims. (Cl. 83-94) 241-22

My invention relates to a new and useful process of grinding materials and particularly minerals which must be ground to a fine state or pulverized or powdered, such as cement, gypsum 5 plaster, raw materials of cement, pigments, etc.

The process is substantially the same regardless of the material which is to be ground considering the dry grinding operation as distinguished from a wet grinding operation. In the present description, the carrying out of the process may be described in connection particularly with the grinding of cement or the raw materials of cement and this description will be found to be ample for enabling those skilled in the art to 10 carry out the process in the grinding of other materials by a dry grinding process.

In the dry grinding process, it has been experienced that the material being ground has a tendency to cling to the surfaces of the grinding media, and also has a tendency to cohere. This adhesion and cohesion result in a cushioning effect, thus decreasing the efficiency of the grinding apparatus as well as its capacity. To overcome this adhesion and cohesion is an object of 20 the present invention. It is also an object of the present invention to provide a process whereby material may be ground in the dry grinding process so that a maximum efficiency of the grinding apparatus may be attained, a greater 25 capacity procured, and a finer grinding of the material made possible.

When the particles of the material to be ground, as they are ground, and particularly as the material is reduced to a powdered or pulverized 30 state, can be maintained in a segregated state, the gathering of the material into flakes in the grinding apparatus will be obviated with an overcoming of the disadvantage of such a "flaking." A part of the process, therefore, consists in introducing to the material being ground a segregating agent and in this regard the word "segregating" 35 is used to indicate that the various particles of the ground materials are brought to such a state as to overcome the tendency to cling together.

In addition to overcoming the cohesion between the various particles, this segregating agent should also have the attribute of preventing adherence of the ground material to the grinding apparatus.

As the material to be ground is fed to the grinding apparatus, and in the grinding of cement, gypsum plaster and cement forming materials, this feeding is constant, there is fed to the feeding apparatus with the material to be ground, a segregating agent, this feeding being preferably 50

constant and preferably in a predetermined constant volume or amount. The segregating material is mixed with the material to be ground during the grinding operation. I have found that a very satisfactory segregating material consists 60 of resin or resinous materials. The term resinous materials is used in a sense not determinative of the physical composition or chemical constituents of the material but the word "resinous" is used in the sense that the adjective is used in 65 classifying dielectric substances.

In the grinding of materials in accordance with this process, I have found that the use of a diffusing material which will serve to readily transmit the segregating agent uniformly 70 throughout the material to be ground is quite desirable and to this end I mix with the material to be ground a diffusing agent. This diffusing agent may consist of any suitable material but 75 I have found that either plaster of Paris or hydraulic cement is most efficient for the purpose. Although the segregating material may be mixed alone with the material to be ground, I prefer to mix the pulverized resin with a diffusing agent such as plaster of Paris or hydraulic cement and 80 then add to this mixture a sufficient quantity of water to set the mixture, after which it may be delivered to the material to be ground, either in its formed state or in a crushed condition. The use of the diffusing agent is particularly 85 desirable in cement as it serves to co-mingle the segregating agent with the ground material and form a homogeneous mixture. The use of a diffusing agent such as described, also overcomes any excessive water repellent characteristics of the ground co-mingled materials. It is believed obvious that when a resinous material 90 is to be ground the segregating agent would necessarily be of a vitreous nature. Furthermore, 95 by introducing the segregating agent with the diffusing material, in addition to the advantages named, there becomes a uniform diffusion of the segregating agent in the material to be ground at an earlier stage in the grinding process which 100 is a distinct advantage in grinding a material of this kind.

The quantity of the segregating agent to be used as well as the quantity of the diffusing agent will depend upon the nature of the material to be ground and can easily be ascertained by a skilled artisan or engineer working in this trade. In the manufacture of cement, I have found that a mixture of one part of resin to five parts of plaster of Paris or hydraulic cement 110 forms a desirable and efficient proportion be-

tween the diffusing agent and the segregating agent. I have also found that a mixing of one part of the mixture of segregating agent and diffusing agent described with two hundred parts 5 of cement will form a satisfactory mixture for the purposes intended. It will be noted that the materials used are less resistant to abrasion than the material to be ground.

By the use of the process, the material may 10 be ground to a finer consistency and the same volume of production maintained with the same power consumption or the material may be ground to the same consistency with an increased 15 volume production while the same power consumption is maintained.

What I claim is:

1. A process of grinding materials consisting

in mixing a segregating agent and a diffusing agent together and delivering the same to the material to be ground during the grinding operation and grinding the whole together.

2. A process of grinding materials consisting in mixing a segregating agent and a diffusing agent together and delivering in a constant delivery the same to the material to be ground during the grinding operation and grinding the whole together.

3. In the grinding of materials for the formation of a hydraulic cement, the process consisting in delivering a resinous material to and grinding the same with the cement-forming materials.

JOHN H. LUNDTEIGEN.

20

95

25

100

30

105

35

110

40

115

45

120

50

125

55

130

60

135

65

140

70

145

75

150